

## UNITED STATES PATENT OFFICE.

ALBIN VUILLERMET AND CEASAR VUILLERMET, OF PHILADELPHIA, PENNSYLVANIA.

## METHOD OF MAKING MOTHER-OF-PEARL TILING.

1,302,252.

Specification of Letters Patent. Patented Apr. 29, 1919.

No Drawing.

Application filed February 13, 1918. Serial No. 216,980.

18-48.8

To all whom it may concern:  
 Be it known that we, ALBIN VUILLERMET and CEASAR VUILLERMET, subjects of the King of Italy, residing at 751 S. Watts St. and 1410 Montrose, respectively, Philadelphia, in the county of Philadelphia and State of Pennsylvania, have invented new and useful Improvements in Methods of Making Mother-of-Pearl Tiling, of which the following is a specification.

The invention relates to a method of making or producing a tiling, slab, brick, or other form of plaque or slab, by the use of mother of pearl as an artistic embellishment or finish for the article, acting also as a binder for the other products employed therewith.

Although we are aware of various kinds and forms of methods of making slabs, ceramics, mosaics and other stone finishes, with various kinds of materials, such as gravel, stone, or the like, we aim to provide an entirely new and novel method of assimilating with cement, a product which by reason of its inherent quality to act as a binder with the cement, also is inherently artistic, novel and beautiful in appearance, and it is to this end that we have devised a method forming a tile or slab with mother of pearl as the basic medium, in order to provide a tile or stone that will have a novel, artistic and refined appearance, withstand wear and tear of the elements, and adapt itself to all forms of architecture and design.

In the promulgation of our method we use, as mentioned heretofore, the hard, pearly internal layer of various kinds of shells, such as pearl oyster, river mussels, and abalone shells, and in order to obtain the desired part thereof for the artistic production of the brick or tile, we crush shells of this character to derive that brilliant and lustrous part of the shell which is usually found in the mantle, or between the mantle and shell proper, and which is generally known as mother of pearl. We may crush these shells by means of any suitable crushing machinery or by hand, to obtain a promiscuous lot of mother of pearl of various shapes and designs, and after doing so we mix the mother of pearl shell with plain cement or hydraulic cement. The plastic mass is now placed in any convenient form of mold to bring about a brick or tile of a desired shape and configuration, and when the same has become set it is removed from the mold and turned up-

side down to expose the plane or other surface, which is ultimately to become the finished surface of the tile or brick.

It will be clear that in forming a brick in the manner mentioned, the mother of pearl will appear on the surface of the brick, and the brick will be thoroughly impregnated therewith, so that the mother of pearl not only is adapted to the ornamental finish and appearance of the brick, but forms the binder with the cement which makes the brick hard and strong, and capable of great use and wear and tear without breaking or cracking. It is of course understood that we may merely form a surface or layer of the mother of pearl for the finished face of the brick, and behind this, mixed with the cement to form an integral part of the brick, we may use the remaining parts of the pearl oyster or mollusk shell which inherently possess an artistic appearance.

However, when the brick or tile has been removed from the mold, and the surface exposed that is later to become the plane and finished surface of the brick, we subject this surface to the action of carborundum wheels or other grinding elements, to not only plane down the surface of cement but also plane down and polish off the exposed and projecting faces or edges of the mother of pearl, so that ultimately when the grinding operation is complete, there will be presented a plane, smooth surface impregnated with numerous bits, particles and pieces of mother of pearl, whose surfaces are plane with the plane surface of cement, and thus the grinding elements not only provide this desired plane surface, but also face off or polish the exposed mother of pearl to provide the artistic finish and result desired.

This surface is now subjected to repeated coats of white damar, not only for the purpose of making the tile waterproof and impervious to moisture, but to finish off the dull appearance of the cement, and also bring about a more desirable polish and higher luster of the mother of pearl.

We may, if desirable, when we first place the plastic mass in a mold, arrange pieces of mother of pearl in the bottom of the mold in fanciful shapes and figures, such as, star designs or fleur de lis, as the case may be, and then, if desirable, use a cement impregnated with pigment, so that the complete and finished surface that will be later exposed, will present an artistic finish resem-

bling a mosaic or ceramic, and thus producing a tile that may be employed in lieu of terra cotta, and used for various purposes, such as, furniture tops, baseboards, and other border work.

Still further, in view of the slight curvature that pearl shell usually has, we may crush the pearl shell carefully or stamp out from the main body thereof, cup-shaped pieces of the mother of pearl from the mantle or interior of the shell, and then carefully dispose these cup-shaped pieces in the bottom of the mold, so that ultimately when the finished surface is ground down by the 10 carborundum wheels or grinding agents, the grinding down of these cup-shaped pieces will form concentric circles of mother of pearl, due to the peculiar formation of pearl shell and the peculiar manner in which 15 20 mother of pearl is formed with pearl shell.

Needless to say a brick or tile produced in the manner mentioned heretofore, will present a neat and artistic finish that cannot be obtained with gravel, stone or other formations 25 of stone structure, that we know have been used heretofore in the formation of ceramics and mosaics, and that it is the inherent quality of mother of pearl to produce a novel surface in a tile or brick, when made 30 as described, so that it will appear very unlike the usual stones or slabs that have repeatedly been employed heretofore, and by reason of the finish of white damar, we not only obtain a tile or brick or slab that will 35 be impervious to moisture, but which also will have a distinct luster, not only of the surface of the cement body, but also of the surfaces of the mother of pearl.

We do not employ mother of pearl or 40 pearl shell in the formation of our brick or

tile merely because of the cheapness of a brick so made, for the reason that pearl shells in the manufacture of buttons and the like are of no further use when the button bodies have been stamped therefrom, but 45 aside from the cheapness of a brick or tile of this character, we rely upon the mother of pearl, because of its inherent quality, luster, brilliant appearance, hardness and susceptibility to polish, to produce a brick or 50 tile that presents a distinct, new and highly ornamental piece of decorative stone work, whose mottled and brightly polished appearance, is highly attractive to the eye, and stands for something different and distinct from the ordinary stone and brick compositions that have been used heretofore in the manufacture of tiling, terra cotta, mosaics, ceramics and other forms of plastic 55 stone and cement products.

Having described our invention, we claim: The herein described method of producing a shell and cement tile or slab, consisting in crushing a quantity of shells to obtain therefrom the mother-of-pearl, thoroughly mixing the mother-of-pearl with a plastic mass of cement to insure the cement being thoroughly impregnated with the pieces of mother-of-pearl, molding this mass into the slab or tile, grinding the 60 surface of the slab or tile to smooth off the rough particles of cement and polish and smooth out the exposed mother-of-pearl and subjecting the finished surface of cement and mother-of-pearl simultaneously to a coat of 65 70 75 white damar.

In testimony whereof we affix our signatures.

ALBIN VUILLERMET.  
CEASAR VUILLERMET.